

# United States Patent Office

2,728,659

Patented Dec. 27, 1955

1

2,728,659

## N-ALKYLHYDROQUINONE ANTISTAIN AGENTS

Anthony Loria, John R. Thirle, and Arnold Weissberger,  
Rochester, N. Y., assignors to Eastman Kodak Company,  
Rochester, N. Y., a corporation of New Jersey

No Drawing. Application June 3, 1953,  
Serial No. 359,422

1 Claim. (Cl. 95—6)

This invention relates to color photography and particularly to a method for preventing the formation of color fog or stain in photographic emulsions.

The method of color photography in which color-forming or coupler compounds combine with the development product of aromatic amino photographic developers to produce dyes is well known. The color formers or couplers may be added directly to the emulsion layers or may be incorporated in the developing solution as described in Fischer U. S. Patent 1,102,028, granted June 30, 1914, or they may be incorporated in a water-permeable medium which is insoluble in the carrier for the sensitive silver salt as described in Mannes and Godowsky U. S. Patent 2,304,940, December 15, 1942, and Jelley and Vittum U. S. Patent 2,322,027, granted June 15, 1943.

A difficulty frequently encountered in these processes is the formation of color fog or stain. When the exposed material is developed in a color-forming developer, dye fog is frequently formed in the emulsion layer. This is because the developing agent has been oxidized to some extent by the action of the air and the oxidized developer tends to couple with the color-forming compound at places in the photographic material where no silver image is produced. It is well known that in these processes the dye should be formed only where the silver halide is reduced to metallic silver, thereby oxidizing the developing agent to a form which couples with the color former. Once the developing agent is oxidized, it couples immediately with the color former whether a photographic image is present or not. Aerial oxidation of the developer or oxidation by means other than the photographic image therefore converts the developer to a form which will immediately react with the color former to produce a color fog or stain. This effect is especially noticeable in materials having couplers incorporated in the sensitive layer since there is no coupler in the developing solution to react with any developing agent which is oxidized by the action of the air. Fog or stain arising from these causes is not readily controlled by the same procedures used to control silver fog.

The control of color fog or stain by incorporating hydroquinone or certain of its derivatives in photographic emulsions is described in Vittum and Wilder U. S. Patent 2,360,290, granted October 10, 1944. Hydroquinones described therein include diamyl hydroquinone and di-octyl hydroquinone. The dialkyl hydroquinones available at that time were the di-secondary and di-tertiary hydroquinones. For example Königs and Mai, Ber. 25, 2649 (1892) describes the preparation of 2,5-di-tertiary amylhydroquinone by the reaction of hydroquinone with isoamylene. Tertiary octyl hydroquinone is described in Niederl U. S. Patent 2,008,032 and Robinson and Hester U. S. Patent 2,008,337. 2,5-di-tertiary octyl hydroquinone has the structure:



2

While 2,5-di-tertiary octyl hydroquinone has good stain-preventing properties when incorporated in photographic color films, it suffers from the disadvantage, when used in silver halide emulsion layers, of causing instability of the color-developed dye to heat or light. This disadvantage will be discussed more fully hereinafter.

It is an object of the present invention to provide antistain agents which cause less instability of the color-developed dye image to heat and light. A further object is to provide antistain agents which are easily compatible with and non-diffusing in the colloid of the photographic layer in which they are incorporated. A further object is to provide antistain agents which are non-diffusing in the photographic layer and which are strong enough reducing agents to react rapidly with oxidized color developer. A further object is to provide antistain agents which do not form highly colored oxidation products when the material containing them is put through an oxidizing bath. Other objects will appear from the following description of our invention.

These objects are accomplished by the use in an emulsion layer or other layer of a photographic material, especially a silver halide emulsion layer in which a colored image is formed by development in a color-forming developer, of a normal alkyl hydroquinone having the formula:



where R is a normal alkyl group having from 5 to 18 carbon atoms, e. g., amyl, hexyl, heptyl, octyl, octadecyl, etc., and R' is hydrogen or the same as R, and is attached to the hydroquinone in the 5 or 6 position.

The following compounds are illustrative of those which we may use:



2-n-octyl hydroquinone



2-n-dodecyl hydroquinone



2-n-octadecyl hydroquinone



2,5-di-n-octyl hydroquinone



The preparation of the compounds of our invention is illustrated by the following examples. In general, the normal alkyl group is introduced by treating hydroquinone with a straight-chain saturated fatty acid, e. g. caprylic acid, in the presence of boron trifluoride, and reduction of the resulting acylhydroquinone to the alkyl hydroquinone.

*Compound 1.—2-caprylylhydroquinone*



A 3-liter, 3-neck flask was charged with a mixture of 220 g. (2 moles) of hydroquinone, 433 g. (3 moles) of n-caprylic acid, and 500 ml. of s-tetrachloroethane. The flask was fitted with a gas-inlet tube extending to the bottom of the flask, a thermometer, and a gas-outlet tube to the hood, and was counterpoised on a balance pan. Gaseous boron trifluoride from a cylinder was then passed directly into the slurry. A yellow color developed and the temperature rose markedly; the rate of addition was regulated to keep the temperature at 50–55° C. without external cooling. The addition was continued until 250 g. (3.7 moles) of boron trifluoride had been absorbed; about three hours was required. The flask should occasionally be swirled by hand during the addition. The reaction mixture gradually formed a deep-yellow solution, from which a yellow solid separated towards the end of the addition. When the absorption was complete, the inlet and outlet tubes were replaced by solid stoppers and the thermometer by an air-condenser protected by a Drierite tube. The flask was left standing overnight (16–20 hours) at room temperature.

The next morning, the flask was heated on a steam bath for 5–6 hours. After a short time, the mixture, which sets to an orange-yellow mush overnight, formed a deep, orange-red solution and drops of water were apparent in the upper part of the flask. At the end of the heating period the mixture was cooled to room temperature with a stream of cold water. It was then poured, with mechanical stirring, into a room-temperature solution of 615 g. (7.5 moles) of sodium acetate in 3100 ml. of water in a 5-liter, 3-neck flask. An additional 100 ml. of tetrachloroethane was used for rinsing the reaction flask. The mixture was then stirred at room temperature for 30–40 minutes to complete the hydrolysis.

The organic layer was allowed to settle and the supernatant aqueous layer removed as completely as possible by decantation with suction. The tetrachloroethane solution was washed twice with 2–3 liters of water, by stirring and decantation as above. Finally, about 2 liters of water were added and the mixture steam-distilled to remove the tetrachloroethane and as much as feasible of

the excess caprylic acid. About 10 liters of distillate was collected.

The residue was cooled to room temperature or below with a stream of cold water; the product crystallized to a somewhat oily yellow-brown solid. This was collected on a large Buchner funnel, and sucked and pressed fairly free of water and most of the adhering oil. Then, without further drying, it was washed with petroleum ether until completely free of oil. About 500 ml. in portions, 10 was required. The crude product formed yellow crystals, M. P. 84–86° C., with preliminary softening at about 75° C. The crude yield was 361 g. (76.5%).

For purification, the material was recrystallized from a mixture of 4 volumes of methanol and 1 volume of water, 15 using 5 ml. per gram, with the addition of Darco (absorbent carbon). The recovery was 327 g. of bright yellow crystals, M. P. 84.5–86° C., with some softening at about 80° C. This amounts to a yield of 69% of the theoretical 472 g.

*2-n-octylhydroquinone*



In a 500-ml., 3-neck flask, with standard-taper ground joints, were placed 23.6 g. (0.1 mole) of 2-caprylylhydroquinone and 2 g. of 10% palladium-on-charcoal catalyst. The air in the flask was replaced by nitrogen, and 200 ml. of glacial acetic acid was added. The flask was then fitted with a fritted-glass gas-introduction tube extending to the bottom of the flask, a moderately high-speed (1700 R. P. M.) propeller or centrifugal stirrer fitted with a rubber seal, and an air condenser with the outlet connected to a glass tube dipping into a cylinder of water so that the reaction flask was under a pressure of 12 to 14 inches of water.

The stirrer was started and hydrogen gas from a cylinder was passed into the reaction mixture at such a rate that the full pressure determined by the depth of the outlet tube in the cylinder of water was maintained in the flask. (A very slow stream of bubbles in the water cylinder indicates a safe rate. The speed of reduction may be estimated by shutting off the hydrogen at the inlet and observing the rate at which the water rises in the exit tube due to the absorption of the hydrogen in the flask. When the water no longer rises at all, the reduction may be considered complete.) The reaction was usually allowed to run overnight (about 20 hours), but some experiments have indicated that 8 to 12 hours might be sufficient.

The catalyst was removed by gravity filtration, and the flask and filter rinsed with 25 ml. of glacial acetic acid. The light-yellow filtrate was heated to boiling and treated with small portions of zinc dust until no further decolorization occurred (2–3 g.). The zinc dust was filtered off and washed with 25 ml. of hot glacial acetic acid. The almost colorless (very light yellow) filtrate and washings were treated with 250 ml. of hot water, mixed thoroughly, and cooled to 0° C. The at-first oily precipitate soon crystallizes to a white solid. This was collected on a Buchner funnel, washed thoroughly with water, and dried in a vacuum desiccator. The product still contained a small amount of oily impurity which was removed by slurring with 50 ml. of petroleum ether, filtering, and washing on the funnel with 50 ml. of petroleum ether in portions.

The 2-n-octylhydroquinone formed a slightly off-white crystalline powder, M. P. 96.5–98° C., with some pre-

liminary softening at 94° C. Yield: 19 g. (85.6% of the theoretical 22.2 g.).

*Compound 4.—2-caprylyl-5-n-octylhydroquinone*



A one-liter, 3-necked flask was charged with a mixture of 111 g. (0.5 mole) of 2-n-octylhydroquinone, 108 g. (0.75 mole) of n-caprylic acid and 250 ml. of s-tetrachloroethane. The flask was fitted with a gas inlet tube extending to the bottom of the flask, a thermometer, and gas outlet tube to the hood. The whole apparatus was counterpoised on a balance pan. Boron trifluoride from a cylinder is passed directly into the slurry at such a rate that the temperature was maintained at 40–45° C. Considerable heat was evolved and the n-octylhydroquinone slowly dissolved to form a dark, yellow-brown solution. When about 62 g. (0.9 mole) of boron trifluoride had been absorbed which required about 1 1/4 hours, the addition was stopped. The outlet and inlet tubes were replaced by solid stoppers and the thermometer by an air condenser protected by a Drierite tube, and the flask left at room temperature overnight (16–20 hours).

The flask was then heated on the steam bath for 6 hours. The mixture soon became turbid and drops of water were apparent in the upper part of the flask. At the end of the heating period the mixture was cooled to room temperature and poured, with stirring, into a room temperature solution of 140 g. (1.7 moles) of sodium acetate in 1260 ml. of water. An additional 50 ml. of s-tetrachloroethane was used for rinsing out the reaction flask. The mixture was stirred at room temperature for about 30 minutes to complete the hydrolysis.

The organic layer was allowed to settle and was separated; the aqueous layer was extracted in a separatory funnel with two 500-ml. portions of ether. The ether extracts and the tetrachloroethane solution were combined, washed once with 250 ml. of water and then with four 250-ml. portions of 5% sodium carbonate solution. The at-first dark, yellow-brown solution became light-yellow on treatment with the carbonate. It was finally washed with 500 ml. of water and dried overnight over magnesium sulfate.

The filtered solution was concentrated under reduced pressure on the steam bath to a volume of about 300 ml. 600 ml. of petroleum ether was added and the mixture cooled to 0° C. The precipitate was filtered off, washed free of dark, oily material with petroleum ether, and dried in the air. It formed yellow crystals, M. P. 82–83° C., with some preliminary softening at 79° C. Weight: 115 g.

A second crop was obtained by concentrating the combined filtrate and washings under reduced pressure on the steam bath to complete removal of the solvents. The dark oily residue was treated with 300 ml. of petroleum ether and left overnight in the ice box. The solid was filtered off and washed with petroleum ether to give 13 g. of yellow crystals, M. P. 81–82° C., softening at 77° C.

The combined crops (128 g.) were recrystallized from 640 ml. of cyclohexane, cooling the filtered solution overnight at about 5° C. The precipitate was filtered off, washed with a little cold cyclohexane and then with three 100-ml. portions of petroleum ether. After drying in the air, the product formed light-yellow crystals, M. P.

82–83° C. with slight softening at 80° C. Yield: 122 g. (70% of the theoretical 174 g.).

*2,5-di-n-octylhydroquinone*



In a 3-liter, 3-necked flask with standard-taper ground joints were placed 69.6 g. (0.2 mole) of 2-caprylyl-5-n-octylhydroquinone and 5 g. of 10% palladium-on-charcoal catalyst. The air in the flask was replaced by nitrogen, and 1 liter of glacial acetic acid was added. The flask was then fitted with a fritted-glass gas-introduction tube extending to the bottom of the flask, a moderately high-speed (1700 R. P. M.) propeller or centrifugal stirrer fitted with a rubber seal, and an air condenser with the outlet connected to a glass tube dipping into a cylinder of water so that the reaction flask was under a pressure of 12 to 14 inches of water.

The stirrer was started and hydrogen gas from a cylinder was passed into the reaction mixture at such a rate that the full pressure determined by the depth of the outlet tube in the water cylinder was maintained in the flask. (A very slow stream of bubbles in the water cylinder indicates a safe rate. The speed of reduction may be estimated by shutting off the hydrogen at the inlet and observing the rate at which the water rises in the exit tube due to absorption of hydrogen in the flask. When the water no longer rises at all, the reduction may be considered complete.) A period of 20 to 22 hours was required; this may conveniently be overnight. Toward the end of the reaction, a bulky white precipitate formed in the flask.

When the reaction was complete, the reaction flask was warmed on the steam bath to 50° C.–60° C., with continued stirring and hydrogen introduction, until the white precipitate redissolved. Excessive or prolonged heating should be avoided. The catalyst was filtered off by gravity and washed with 100 ml. of hot glacial acetic acid. The initial filtrate was colorless, but some yellow color developed toward the end of the filtration and during the washing. The light-yellow filtrate and washings were heated on the steam bath and treated with small portions of zinc dust until no further decolorization resulted. About 5 g. was used. The zinc dust was then removed by filtration and washed with a little hot glacial acetic acid.

The almost colorless filtrate was treated slowly, with stirring, with 1 liter of hot water. A white precipitate formed. The mixture is cooled to about 10° C. The precipitate was filtered off and washed thoroughly with water. After drying in a vacuum desiccator at room temperature, it formed a very slightly off-white powder, M. P. 80, 104–109° C. The weight was 66 g.

Recrystallization from 660 ml. of cyclohexane, followed by washing with 25 ml. of cold cyclohexane and three 100-ml. portions of petroleum ether, yielded 60 g. (90%) of white plates, M. P. 109.5–110.5° C., with some preliminary softening at 106° C.

*Compound 6.—2-caprylyl-4-methoxyphenol*

Boron trifluoride was passed into a mixture of 124 g. (1 mole) of p-methoxyphenol, 216 g. (1.5 moles) of caprylic acid, and 300 cc. of dry tetrachloroethane for a

period of about four hours. The reaction mixture was allowed to stand overnight at room temperature and was then heated on a steam bath for about three hours. When cool, the mixture was poured into 130 g. of sodium acetate in 2 liters of water with stirring. The layers were separated and the water layer extracted with ether. The ether extract was combined with the tetrachloroethane, washed thoroughly with water, and concentrated under reduced pressure. The 2-caprylyl-4-methoxyphenol was collected at 195°/10 mm. (yield 181.5 g.). Recrystallization from about 600 cc. of methanol gave 137 g. (55%), M. P. 42.5-44°.

#### 4-methoxy-2-n-octylphenol

Three portions of 2-caprylyl-4-methoxyphenol, totaling 170 g., were hydrogenated using for each approximately 170 cc. of glacial acetic acid, 10-12 g. of 10% palladium on charcoal, and hydrogen at 30-40 p. s. i. The reduction was performed in a Parr hydrogenation apparatus at room temperature and was complete overnight. The catalyst was filtered off and the filtrate poured into a large volume of water. The organic material was extracted into ether, and the ether layer was neutralized with sodium bicarbonate, washed with water, dried over sodium sulfate, and concentrated. The 4-methoxy-2-n-octylphenol was collected at 187-190°/10 mm. (yield 141 g.; 88%).

#### 2-caprylyl-4-methoxy-6-n-octylphenol

Eighty grams (0.339 mole) of 4-methoxy-2-n-octylphenol, and 65 grams (0.45 mole) of caprylic acid were dissolved in 150 cc. of dry tetrachloroethane, and boron trifluoride was passed in for about 6 hours. The mixture was heated on a steam bath for about 5 hours and then, on cooling, was poured into a large quantity of water and treated with excess sodium carbonate. Ether was added to aid separation and then the ether layer was washed thoroughly with water. The ethereal solution was concentrated, and the forerun removed up to B. P. 240°/10 mm. The product (79 g.; 64%) was collected at 195-205°/1 mm. Crystallization from 95% alcohol gave 52.5 g. (42.5%), M. P. 30-31°.

#### 2,6-di-n-octyl-4-methoxyphenol

Three portions totalling 167 g. (0.461 mole) of 2-caprylyl-4-methoxy-6-n-octylphenol were reduced catalytically in a Parr hydrogenation apparatus. Each portion was dissolved in about 250 cc. of glacial acetic acid and used approximately 15 g. of 10% palladium on charcoal with hydrogen at 30-40 lbs. per sq. in. Reduction occurred quite slowly (ca. 20 hours) and gentle warming was required. After filtering off catalyst, the filtrate was poured into a large quantity of water and extracted with ether. The ether extract was neutralized with sodium carbonate, washed with water, dried over sodium sulfate and concentrated. 2,6-di-n-octyl-4-methoxyphenol was collected at 190-200°/1 mm. (yield 142 g.; 88.5%; M. P. 39-41°).

#### 2,6-di-n-octylhydroquinone

Twenty-five grams of 2,6-di-n-octyl-4-methoxyphenol was hydrolyzed by refluxing in a mixture of 400 cc. of glacial acetic acid and 80 cc. of hydrobromic acid (48%) for approximately 24 hours. When cool, the reaction mixture was poured into at least twice its volume of water and chilled under running water for a few hours. The solid was filtered off and the sticky material was slurried carefully in the funnel with ice-cold petroleum ether, most of the color and stickiness being removed by this procedure. The product was recrystallized from a mixture of approximately 215 cc. of ligroin (B. P. 90-120°) and 215 cc. of low-boiling petroleum ether, giving 15.5 g. (64%), M. P. 81.5-82.5°.

The 2,6-di-n-octylhydroquinone can also be prepared as follows:

#### 4-nitro-2,6-di-n-octylphenol

In a 200-ml. flask were mixed 5.64 g. (0.02 mole) of 10-nona-decanone (J. A. C. S., 55, 1697), 2.5 g. (0.02 mole) sodium nitromalonaldehyde (Amer. Chem. J., 22, 4), 75 ml. of absolute ethyl alcohol, and 5 g. of potassium hydroxide dissolved in 40 ml. of water. The flask was equipped with a water-cooled condenser and the mixture refluxed on a steam bath for 18 hours. The reaction mixture was cooled to about 20° C. and the small amount of colorless precipitate that formed was filtered and washed on the funnel with 25 ml. of cold water. The filtrate and the wash water were combined and evaporated to about 50 ml. and let stand overnight. The yellow crystalline precipitate that formed was filtered and washed on the funnel with 25 ml. of ice-cold water. It was suspended in 100 ml. of 50 percent aqueous alcohol and acidified with 4 ml. of dilute hydrochloric acid. The colorless solid that formed was collected and crystallized twice from acetonitrile. There was obtained 4.1 g. of product melting at 75-76° C.

#### 2,6-di-n-octylquinone

The 4-nitro-2,6-di-n-octylphenol was reduced to the amino compound using Raney nickel catalyst and 10 ml. of 30 percent sodium dichromate in water was added dropwise to an aqueous acetone solution of the 2,6-di-n-octyl-4-aminophenol (2.2 g. in 100 ml. of acetone + 50 ml. of water) at room temperature with mechanical stirring. After 3 hours, the acetone was evaporated under reduced pressure, and water was added to the residue. The oily yellow solid formed was taken up in ether; the ether solution was washed with water, dried over sodium sulfate, and the solvent evaporated. The yellow solid residue melted at 57-60° C.

#### 2,6-di-n-octylhydroquinone

An acetic acid solution of 2,6-di-n-octylquinone (2.2 g. in 50 ml.) was heated to reflux and while stirring 3 g. of zinc dust was added to it in small portions. After 30 minutes' refluxing, the excess zinc was removed by filtration, and the filtrate was added to 200 ml. of cold water. The mixture was allowed to stand overnight; the precipitate that formed was filtered, washed well with water, and air-dried. The dried product was crystallized three times from petroleum ether, B. P. 30-60° C. There was thus obtained a white crystalline solid melting at 82-83°, which, on standing, turns to a pink color.

#### Compound 2.—2-n-dodecylhydroquinone

2-n-dodecylhydroquinone (M. P. 106.5-108° C.) was prepared as described by Cook, Heilbron, and Lewis, J. Chem. Soc., 1942, 659, with certain modifications, e. g., reduction of the intermediate ketone with palladium-on-charcoal catalyst.

#### Compound 3.—2-n-octadecylhydroquinone

2-n-octadecylhydroquinone (M. P. 114-115° C.) was prepared as described by Cook, Heilbron, and Lewis, J. Chem. Soc., 1942, 659, reducing the intermediate ketone, however, with palladium-on-charcoal catalyst.

#### Compound 5.—2,5-di-n-dodecylhydroquinone

2,5-di-n-dodecylhydroquinone was prepared from 2-n-dodecylhydroquinone by acylation with lauric acid as described above for 2-caprylyl-5-n-octylhydroquinone. The ketone (M. P. 88-90° C.) was reduced by hydrogen and palladium-on-charcoal catalyst giving 2,5-di-n-dodecylhydroquinone. (M. P. 108-110° C.)

The antistain agents of our invention are useful, in general, with emulsions containing couplers incorporated in the manner described in Mannes and Godowsky U. S. Patent 2,304,940 or Jelley and Vittum U. S. Patent 2,322,027.

Couplers such as those described in Weissberger U. S. Patent 2,298,443 and Salminen and Weissberger U. S.

Patent 2,423,730, when incorporated in this way, produce dyes upon color development which are prone to fading by the action of visible or ultraviolet light, when known antistain agents such as 2,5-di-tert. octyl hydroquinone are used in the emulsion layer. These are the yellow and cyan dyes. The magenta dyes, such as those formed from couplers described in Loria, Weissberger and Vittum U. S. Patent 2,600,788 are relatively little affected by the known antistain agents upon the action of light.

In order to illustrate the effect of our antistain agents, 10 the following test was made.

A quantity of the antistain agent, the molar equivalent of 0.05 g. of 2,5-di-tert. octyl hydroquinone, was dissolved with 0.5 g. of coupler in 1.5 cc. of dibutylphthalate. To this solution was added 11 cc. of 10% gelatin solution and 2.8 cc. of 5% Alkanol B (sodium alkyl naphthalene sulfonate) solution. The mixture was passed through a colloid mill three times, and to the resulting dispersion, 32 cc. of a gelatino-silver halide emulsion were added, and the mixture blended and coated on a film support so that the anti-stain agent was equivalent to 5 mg. per sq. ft. of 2,5-di-tert.-octyl hydroquinone.

Two check coatings were made; one containing no anti-stain agent, and one containing 5 mg. per sq. ft. of 2,5-di-tert. octyl hydroquinone.

The film strips were exposed on a 1b sensitometer using a silver wedge varying in density from 0 to 3. They were then developed 10 minutes at 68° F. in the following developer:

|                                    |    |       |
|------------------------------------|----|-------|
| 2-amino-5-diethylamino toluene HCl | 2  | G. 30 |
| Sodium sulfite (desiccated)        | 2  |       |
| Sodium carbonate, monohydrate      | 20 |       |
| Potassium bromide                  | 2  |       |
| Water to 1 liter.                  |    |       |

This was followed by 5 minutes in the following stop bath:

|                            |         |    |
|----------------------------|---------|----|
| Sodium sulfite, desiccated | g. 75   | 40 |
| Acetic acid (28%)          | cc. 235 |    |
| Boric acid, crystals       | g. 37.5 |    |
| Potassium alum             | g. 75   |    |
| Water to 1 liter.          |         |    |

After washing, bleaching in ferricyanide-bromide, fixing in 30% hypo solution and again washing, the wavelength-density curves for each coating were read before and after exposure to visible and ultraviolet light. The loss of density at the maximum of the wavelength-density curve after exposure in the Fade-O-Meter for 6 hours and comparison with the check coatings under similar conditions indicated the effect of the agent under test. The following table shows these results:

#### Loss in density at maximum absorption

| Agent                          | Cyan dye | Yellow dye |
|--------------------------------|----------|------------|
| Check (none)                   | 0        | 0          |
| 2,5-di-tert. octylhydroquinone | .25      | .08        |
| Compound 1                     | .01      | +.10       |
| Compound 3                     | .06      | +.10       |
| Compound 4                     | .09      | .04        |
| Compound 6                     | .08      | +.01       |

These results show that in the case of the cyan dye, all of the agents caused less fading than 2,5-di-tert. octyl hydroquinone. In the case of the yellow dye, compounds 1, 3 and 6 showed an increase in density over the standard, and compound 4 produced about half as much loss in density as the standard.

The antistain agents of our invention may also be used in non-sensitive overcoating or filter layers, such as a colloidal silver interlayer of multilayer photographic material. In general, the antistain agents of our invention are used in the emulsion or other layer in quantities ranging from 0.07 gram to 4.3 grams per liter of emulsion or gelatin solution. These values are, however, merely illustrative.

In certain cases the antistain agents of our invention may be incorporated in a processing solution such as a prebath, first developer bath, or color-forming developer used with color film which is developed with a primary aromatic aminodeveloping agent.

Our materials are particularly useful with color-forming emulsions coated on paper supports where it is especially important to reduce the minimum or fog densities. This applies both to negative developed paper and to reversal paper as well as to transparency materials.

It will be understood that the examples and modifications described herein are illustrative only and that our invention is to be taken as limited only by the scope of the appended claim.

We claim:

A color-forming photographic emulsion having reduced fogging tendency, comprising a silver halide emulsion having incorporated therein a non-diffusing coupler compound capable of coupling with the oxidation product of a primary aromatic amino developing agent and as an antistain agent a normal alkyl hydroquinone having the formula



45

where R and R' are normal alkyl groups of from 9 to 18 carbon atoms, and R' is attached to the hydroquinone nucleus in a position selected from the class consisting of 5 and 6 positions.

#### References Cited in the file of this patent

#### UNITED STATES PATENTS

55 2,360,290 Vittum et al. Oct. 10, 1944

60